

# UNITED STATES PATENT OFFICE.

OTTO RÖHM, OF DARMSTADT, GERMANY, ASSIGNOR, BY MESNE ASSIGNMENTS, TO THE CHEMICAL FOUNDATION, INC., A CORPORATION OF DELAWARE.

## PROCESS FOR TANNING WITH ALUMINIUM SALTS.

1,421,723.

Specification of Letters Patent.

Patented July 4, 1922.

No Drawing.

Application filed December 6, 1917. Serial No. 205,880.

To all whom it may concern:

Be it known that I, OTTO RÖHM, a subject of the King of Wurttemberg, residing at No. 4-6. Weiterstädtterstrasse, in the city of 5 Darmstadt, Grand Duchy of Hessa, German Empire, have invented an Improvement in Processes for Tanning with Aluminium Salts, (for which I have filed application in Germany, Oct. 27, 1916); and I do hereby 10 declare that the following is a full, clear, and exact description of the same.

Leather tanned in the usual manner with alum must be treated with water before being dyed, in order to remove superfluous 15 alum and common salt. It is well known that in doing so a part of the tanning substance is washed out of the outer layers of the leather and particularly out of the grain. Owing to this untanning, grain defects arise 20 and the leather becomes insufficiently tanned and hard. In order to avoid this the leather had to be dried and kept for weeks and months in dry condition in order to more intimately unite the tanning substance with 25 the skin.

Now it has been found that this keeping of the leather dried with an excess of tanning substance is not necessary if the skins are treated with a solution of a salt of the lower 30 fatty acids. For this purpose the formates or acetates of the alkalies or earth alkalies, for example sodium formates, come particularly into question.

The treatment with these salts can take 35 place at different stages of the process for producing leather. If the sodium formate is added to the tanning liquor itself the same result is obtained, without having to store the leather in dry condition, as by the usual 40 alum tanning process with this subsequent treatment. Further, the addition of wheat flour usual in making kid leather can either be entirely omitted or it can be replaced by finely powdered mineral substances, such as 45 talcum, etc. Moreover the greasing can be decreased and in many cases entirely omitted.

If the sodium formate is not added to the tanning liquor itself the removal of tanning substances by the washing process after employing the usual alum process can be avoided by placing the moist leather taken 50 out of the tanning liquor into the solution of a salt of the lower fatty acids. If it is desired to retain the usual alum tanning process with the subsequent drying, because 55

the choice of the skins for white, black or colored leather is easier and more convenient in dry condition, the fatty acids are added to the water used for washing the dried alum leather.

60

### Examples.

1. *Tanning with alum + salt + sodium formate + talcum.*—For every 100 kg. of depilated skins from which the liquid has been 65 allowed to strain off 8 kg. alum + 2½ kg. salt + 500 g. sodium formate 10 kg. talcum + 50 l. water are required. In this tanning liquor the skins are moved about for an hour and they are then allowed to lie in the same during the night. In the morning the skins are again moved about for a short time and they are then dried in the usual manner.

2. *Washing of alum tanned moist fur with sodium formates.*—The furs tanned in the 75 usual manner with alum and salt are kept moist for 2 or 3 days of 24 hours and washed with 200% of a 1 or 2% solution of sodium formate, in proportion to the tanning weight, and they are then dried and dressed in the 80 usual manner.

3. *Washing dried alum leather with sodium formate.*—10 kg. of dried alum leather are moved about for half an hour in 50 liters of water of 20° C. until they are entirely 85 soaked. Then 300 g. of sodium formate dissolved in a little water are added, and the leather is moved about again for an hour. In this liquid the skins are allowed to lie for a few hours and they are then dried in the 90 usual manner.

4. *Washing dried furs with sodium formate.*—10 kg. of dried alum tanned furs are placed in 40 to 50 liters of a 1% sodium formate solution or they are moved about in 95 same until they are entirely soaked. They are allowed to lie in this liquid for some time and are then dried in the usual manner.

### Claims.

100

1. The process of tawing which comprises immersing hides or skins in a liquor containing 8 kg. potassium alum, 2½ kg. sodium chloride, 500 g. sodium formate, 10 kg. talcum and 50 l. of water for each 100 kg. of 105 hides or skins.

2. The process of tawing which comprises immersing hides or skins in a liquor containing alum, sodium chloride, sodium formate, talcum, and water.

110

3. The process of tawing which comprises immersing hides or skins in a liquor containing alum, sodium chloride, sodium formate, talcum and water, moving the skins about in said liquor for a short time, allowing to remain in said liquor about fourteen hours, moving about in said liquor again for about one hour, and finally drying.
4. The process of tawing which comprises immersing hides or skins in a liquor containing 8 kg. potassium alum, 2½ kg. sodium chloride, 500 g. sodium formate, about 10 kg. talcum, and about 50 l. of water for each 100 kg. of hides or skins, moving the skins about in said liquor for a short time, allowing to remain in said liquor about fourteen hours, moving about in said liquor again for about one hour, and finally drying.
5. In the process of tawing the step, which comprises the employment of a solution containing a formate of an alkali metal.
6. In the process of tawing the step which comprises the employment of a solution of a formate of an alkali metal and a finely powdered mineral substance.
7. In the process of tawing the step, which comprises the employment of a liquor containing a formate of alkali metal and a finely powdered mineral substance.
8. In the process of tawing the step, which comprises the employment of a formate of an alkali metal, together with talcum.
9. In the process of tawing the step, which comprises the immersing skins in a liquor containing a formate of an alkali metal and a finely powdered mineral substance.
10. In the process of tawing, the step which comprises immersing skins in a solution containing a formate of an alkali metal and talcum.
11. A tanning composition including potassium alum, sodium chloride, sodium formate, talcum and water.

DR. OTTO RÖHM.